

## UNITED STATES PATENT OFFICE

2,663,690

HIGH-TEMPERATURE SODIUM MYRISTATE  
GREASE CONTAINING N,N'DIPHENYL  
PARA-PHENYLENE DIAMINEGeorge W. Eckert, Glenham, N. Y., assignor to  
The Texas Company, New York, N. Y., a cor-  
poration of DelawareNo Drawing. Application February 16, 1951,  
Serial No. 211,446

4 Claims. (Cl. 252—42.1)

1

The present invention relates to sodium myristate greases suitable for the high temperature lubrication of ball and roller bearings. More particularly it relates to sodium myristate greases having improved high temperature performance characteristics which are imparted by small amounts of N,N' diphenyl para-phenylene diamine which they contain.

It has been found that sodium myristate greases have special properties which make them particularly suitable for the lubrication of anti-friction bearings at high temperatures. Besides possessing a dropping point in excess of 400° F. they are resistant to the action of water and provide satisfactory lubrication with negligible change in texture and consistency even at temperatures above 300° F. However sodium myristate greases exhibit a tendency to eventually break down through physical and chemical changes, such as phase separation, when they are employed for the lubrication of ball and roller bearings at high temperatures and at high rotative speeds for a substantial period of time. The antioxidants and other additives which have been employed in other known types of ball and roller bearing greases are generally ineffective in extending the service life of these greases to the desired extent under the conditions of high temperature and high shear stress to which they are subjected in this type of service.

The principal object of this invention is to provide a grease of greatly extended service life for the high temperature lubrication of anti-friction bearings. Another object is to provide a sodium myristate grease having a service life in excess of 1000 hours at 300° F. in anti-friction bearing lubrication.

In accordance with my invention a grease suitable for the lubrication of ball and roller bearings at high temperatures and at high rotative speeds for long periods of time comprises an oleaginous base thickened to a buttery consistency with a fatty acid soap which comprises a predominant amount of sodium myristate, and containing a small amount sufficient to improve the high temperature performance characteristics thereof of N,N' diphenyl para-phenylene diamine. I have found that such greases are markedly superior in high temperature properties both to greases of very different composition and to greases of otherwise similar composition containing additives which have been proposed heretofore for improving oxidation resistance and other properties of ball and roller bearing greases. In particular, the greases of my invention have

2

exceptional lubricating properties for the long time lubrication of anti-friction bearings at temperatures up to 300° F. and at rotative speeds of 10,000 R. P. M. and higher.

The sodium myristate soap which is employed as the thickening agent may be prepared by saponifying a mixture of low molecular weight fatty acids comprising at least 70%, and preferably at least 90%, by weight of myristic acid and/or the glycerides of such acids with caustic soda or other suitable sodium compound, preferably employing a small excess of the alkali sufficient to provide an excess of about 0.1 to about 1% of free alkali in the finished grease. The grease may suitably contain from about 15% to about 25% by weight of this soap.

The N,N' diphenyl para-phenylene diamine may be present in the grease in widely varying amounts depending upon the magnitude of the effect desired. In general, a suitable range will be from about 0.5% to about 8%, and preferably from about 1% to about 5%, by weight based on the weight of the grease.

The oleaginous base may be any high boiling organic oil of lubricating characteristics, such as a mineral oil fraction obtained from a paraffinic, naphthenic or mixed base crude by any of the usual refining methods, an animal or vegetable oil such as lard oil, corn oil, castor oil, or the like, or a synthetic oil obtained by polymerization or chemical condensation reactions, as well as mixtures of these. It may advantageously be a blend of distillate and residual lubricating oil fractions from a paraffin base crude.

In addition to the N,N' diphenyl para-phenylene diamine, other additives may be present in the grease such as extreme pressure agents, antioxidants, anticorrosives, and so forth, so far as no incompatibility exists between them and N,N' diphenyl para-phenylene diamine.

The greases of my invention may be prepared by any of the conventional methods for obtaining greases of the buttery or short fiber type suitable for the lubrication of anti-friction bearings. They are preferably prepared by the method described in the copending application of O. P. Puryear and M. D. Bray, Serial Number 130,588, filed December 1, 1949, now Patent No. 2,542,570, dated February 20, 1951. According to the method of said application, a commercial myristic acid is saponified with a small excess of sodium hydroxide solution in the presence of small amounts of mineral oil and water, the resulting soap base dehydrated at a temperature in the range 295-320° F. and sufficient mineral oil added to obtain

the desired consistency, the mineral oil addition being carried out in two stages so that a total amount of mineral oil equal to at least twice the weight of the fatty acids initially charged is added before the temperature of the mass is allowed to drop below 260° F.

Table I below gives high temperature performance test data obtained on a number of greases prepared according to the above-described method and stabilized by various different types of compounds including N, N' diphenyl para-phenylene diamine. The base oil employed in the preparation of these greases was a 1 to 3 blend of a solvent refined and clay treated paraffinic distillate oil having an API gravity of 29.2, and SUS viscosity at 100° F. of 333 and a COC flash point of 435° F., and a solvent refined, clay and acid treated paraffinic residual oil having an API gravity of 27.9, an SUS viscosity at 100° F. of 1724.7 and a COC flash point of 555° F. The myristic acid employed had a neutralization number of 240, a saponification number of 241 and a titer, °C. of 41.8. The finished greases contained about 20% of the sodium soap prepared from this myristic acid and were slightly alkaline with about 0.3% of free alkali, calculated as sodium hydroxide. The additives were added to the greases at the end of the manufacturing process after the temperature had dropped below about 250° F. The N, N' diphenyl para-phenylene diamine was added in the form of a slurry in a part of the residual base oil.

TABLE  
High temperature performance test

| Additive                                                   | Hours to Failure |         |
|------------------------------------------------------------|------------------|---------|
|                                                            | 425° F.          | 300° F. |
| None                                                       |                  | 219     |
| 1% Hydrazobenzene                                          |                  | 326     |
| 5% 4-methyl-2,6-di-tertiary butyl phenol                   | 24               | 697     |
| 3% Zinc dibutyl dithiocarbamate+2% Ba phenolate            |                  | 358     |
| 8% Hydrazine alkyl salicylate+2% Ba phenolate              |                  | 264     |
| 1% 2,4-di-tertiary butyl phenol+2% Ca isooctyl o-phosphate |                  | 543     |
| 1% Diphenylamine                                           | 23               | 392     |
| 5% Diphenylamine                                           |                  | 428     |
| 3% Diphenylamine+2% 4-methyl-2,6-di-tertiary butyl phenol  |                  | 524     |
| 1% Triphenylbenzidine                                      |                  | 452     |
| 1% p,p'-Diamino di-tertiary methane                        | 9                | 50      |
| 1% s-Diphenylethlenediamine                                |                  | 288     |
| 1% Diethylenetriamine                                      |                  | 251     |
| 5% Isopropoxy diphenylamine                                | 12               | -----   |
| 4% p-Phenylene diamine                                     | 11               | -----   |
| 1% di-b-Naphthyl p-phenylene diamine                       |                  | 645     |
| 5% di-b-Naphthyl p-phenylene diamine                       | 24               | -----   |
| 2.5% N,N' Diphenyl p-phenylene diamine                     | 47               | -----   |
| 5% N,N' Diphenyl p-phenylene diamine                       | 48               | 1056    |

The High Temperature Performance Test of the foregoing table is a test for determining the performance characteristics of greases in anti-friction bearings at elevated temperatures and high rotative speeds. The test unit consists essentially of a steel spindle supported on ball bearings in an electrically heated housing and driven by an electric motor connected into an electric circuit containing a low amperage fuse 0.1 ampere below that required for full load running. The bearings are Norma-Hoffmann ABEC No. 3 grade, and are mounted on the spindle approximately 5 1/2 inches apart, one bearing being the test bearing and the other an outboard guide bearing. A thrust load of 17.5 pounds is applied to the test bearing. The test consists of operating the test bearing for twenty-four hours at 10,000 R. P. M. and at a temperature

of 300° F. or at a temperature between 250° F. and 475° F. followed by a shutdown and cooling period of two hours, and repeating this cycle until the lubricant fails, which is indicated by rupture of the low amperage fuse in the motor circuit. In starting up the test, three grams of the test grease are charged to the test bearing and worked into and around the race and balls; the outboard bearing may be packed with any suitable grease. The bearings are next rotated both clockwise and counterclockwise for one minute each at 200 R. P. M. and assembled into the test unit. The heaters and the motor are then started and the test bearing brought up to the test temperature as rapidly as possible, which requires 1.0 to 1.25 hours for a temperature of 300° F., while the spindle is rotated at a speed of 10,000 R. P. M. After 24 hours of operation the heaters and motors are shut off for 2 hours, during which the temperature of the test bearing drops to a minimum of 120-130° F. The total hours of operation, excluding the two hour shutdown periods, to the failure point is recorded as the "hours to failure." A grease giving satisfactory lubrication for 1000 hours at 300° F. under the conditions of this test is considered a very superior lubricant for the lubrication of anti-friction bearings at elevated temperatures and at high rotative speeds.

As shown by the table, a sodium myristate grease containing N,N' diphenyl para-phenylene diamine gave satisfactory lubrication in anti-friction bearings for over one thousand hours at 300° F. in the High Temperature Performance Test described above. The effect obtained by adding N,N' diphenyl para-phenylene diamine to the sodium myristate grease was almost twice that obtained by any of the other compounds tested, which are usually considered to be effective stabilizing agents for organic lubricating compositions, as well as combinations of such additives and also by closely analogous derivatives of phenylene diamine.

Obviously many modifications and variations of the invention, as hereinbefore set forth, may be made without departing from the spirit and scope thereof, and therefore only such limitations should be imposed as are indicated in the appended claims.

I claim:

1. A ball and roller bearing grease capable of lubricating anti-friction bearings at high rotative speeds for long periods at a temperature of 300° F. containing as the essential constituents a major proportion of an oleaginous liquid lubricating base, about 15-25% by weight based on the grease of a sodium soap of a soap-forming fatty material containing at least 70% based on the fatty material of myristic acid, said soap thickening said lubricating base to a buttery grease-like consistency, and about 0.5-8% by weight based on the grease of N,N' diphenyl para-phenylene diamine.

2. Claim 1 wherein the fatty material contains at least 90% of myristic acid.

3. A lubricating grease consisting essentially of the following ingredients in the approximate specified proportions:

Sodium myristate 15-25%.  
N,N' diphenyl para-phenylene diamine 1-5%.  
Excess NaOH 0.1-1.0%.  
Lubricating oil comprising a blend of a paraffinic distillate oil and a residual oil Remainder.

4. Claim 1 wherein the grease contains about 0.1-1.0% by weight based on the weight of the grease of free alkali, calculated as sodium hydroxide.

GEORGE W. ECKERT. 5

References Cited in the file of this patent

UNITED STATES PATENTS

| Number    | Name             | Date              |
|-----------|------------------|-------------------|
| 1,599,854 | Van Gundy et al. | Sept. 14, 1926 10 |

|  | Name            | Date          |
|--|-----------------|---------------|
|  | Hilliker        | Jan. 29, 1935 |
|  | Adams et al.    | Jan. 21, 1941 |
|  | Woods et al.    | June 13, 1944 |
|  | Woodward et al. | Feb. 20, 1945 |
|  | Vincent         | Aug. 27, 1946 |
|  | Puryear et al.  | Feb. 20, 1951 |